

**United States Patent** [19]  
**Mark**

[11] Patent Number: **4,478,603**

[45] Date of Patent: **Oct. 23, 1984**

[54] **COAL-AQUEOUS MIXTURES COMPRISING  
NONIONIC AND ANIONIC SURFACTANTS**

[75] Inventor: Seymour Mark, Northampton, Pa.

[73] Assignee: The Standard Oil Company,  
Cleveland, Ohio

[21] Appl. No.: **495,628**

[22] Filed: **May 18, 1983**

**Related U.S. Application Data**

[63] Continuation-in-part of Ser. No. 416,606, Sep. 10, 1982,  
, which is a continuation-in-part of Ser. No. 230,062,  
Jan. 29, 1981, Pat. No. 4,358,293.

[51] Int. Cl.<sup>3</sup> ..... **C10L 1/32**

[52] U.S. Cl. ..... **44/51; 44/72;  
44/77; 252/351; 252/DIG. 1**

[58] **Field of Search** ..... **44/51, 77, 72; 252/351,  
252/DIG. 1**

[56] **References Cited**

**U.S. PATENT DOCUMENTS**

**4,392,865 7/1983 Grosse et al.**

*Primary Examiner*—Jacqueline V. Howard  
*Attorney, Agent, or Firm*—Scully, Scott, Murphy &  
Presser

[57] **ABSTRACT**

Coal-aqueous mixtures having high solids content comprising coal, water and a combination of nonionic and anionic surfactants.

**54 Claims, No Drawings**

**COAL-AQUEOUS MIXTURES COMPRISING  
NONIONIC AND ANIONIC SURFACTANTS**

**CROSS-REFERENCE TO RELATED  
APPLICATIONS**

This application is a continuation-in-part of U.S. application Ser. No. 416,606 filed Sept. 10, 1982 which in turn is a continuation-in-part of U.S. application Ser. No. 230,062 filed Jan. 29, 1981, now U.S. Pat. No. 4,358,293, the entire contents of which are incorporated by reference herein.

**BACKGROUND OF THE INVENTION**

The present invention relates to the dispersion of carbonaceous materials and more particularly to coal-aqueous coal mixtures.

Coal as an energy source is in abundant supply. It is estimated that in the United States there is more energy available in coal than in petroleum, natural gas, oil shale and tar sands combined. The substitution of coal for natural gas and oil on a large scale would therefore seem a ready-made solution to our energy problems. Unfortunately, however, unlike oil and gas consumption, coal use is limited not by reserves or production capacity but rather by the extraordinary industrial and regulatory difficulties of burning it in a convenient, efficient and environmentally acceptable manner.

A number of techniques are being explored to provide coal as a more useful energy source. One such technique employs gasification methods such as destructive distillation, to effect the conversion of coal to a low or medium Btu gas. In another approach, high pressure hydrogenation is utilized to liquefy coal to make it more suited for transport, burning and the like.

Another technique suggested, and the one to which the present invention relates, is the technique whereby solid coal particles are dispersed in a fluid carrier medium, such as fuel oil or water to form coal-aqueous or coal-oil mixtures.

Coal-oil and coal-aqueous mixtures, however, are distinct systems, each having its own difficulties of formulation. For example, while coal and oil are relatively compatible, coal and water are not. Thus, unlike in the formulation of coal-oil admixtures, in the formulation of coal-aqueous admixtures, the initial dispersing of the coal in the continuous water phase, especially large amounts of coal, represents a challenging obstacle. Moreover, after dispersion, stabilizing, i.e. keeping the coal from settling out of the water phase, must be also achieved.

Such coal mixtures offer considerable advantages. They are more readily transported than dry solid coal, are more easily stored and are less subject to the risks of explosion by spontaneous ignition, the latter being a significant factor in handling coal. In addition, providing coal in a fluid form can permit its burning in apparatus normally used for burning fuel oil. This can greatly facilitate the transition from fuel oil to coal as a primary energy source, another highly desirable result.

Various coal-oil and coal-aqueous mixtures have been described in the literature. For example, British Pat. No. 1,523,193 discloses a mixture comprised of fuel oil and from 15 to 55% by weight of finely ground coal particles reduced in particle size to 10 microns or finer. The effort required to grind coal to such fine sizes, however, makes the process less economically attractive. More-

over, the use of fuel oil as a carrier medium negates the requirement of lessening our dependence upon fuel oil.

U.S. Pat. No. 4,251,229 is an example of coal-oil mixtures stabilized with high molecular weight adducts of alkylene oxide and an alcohol, an amine, a carboxylic acid or phenol having at least three active hydrogens. In this patent, oil is the continuous carrier phase and accordingly, the stabilization of the coal, as emphasized repeatedly therein, in the continuous oil phase, is essentially the only concern.

U.S. Pat. No. 4,242,098 discloses aqueous coal slurry compositions containing water soluble polymers, which are thickeners, such as xanthan gum, hydroxypropyl guar gum or poly(ethylene oxide) having a molecular weight over 100,000.

In U.S. Pat. No. 3,762,887, there is disclosed a dispersion of coal in an aqueous medium wherein the coal is ground to a defined array of particle sizes, a substantial portion of which being about 325 mesh Tyler Standard screen or even finer. Here again, substantial and selective grinding of the coal is required.

U.S. Pat. No. 4,217,109, discloses a technique for cleaning and dispersing coal in water utilizing dispersing agents which by selective adsorption impart different electrical charges to the carbon particles and the impurities. The dispersing agents taught are polyelectrolytes, such as alkali metal and ammonium salts of polycarboxylic acids and polyphosphates.

PCT International Application No. WO 83/01069 discloses compositions comprising coal, water and polyelectrolytes which are water soluble polyethylenes containing certain sulfur containing substituents. Combinations of these sulfur containing polyethylenes and other surfactants such as polyacrylic acid and poly(ethylene oxides) (exemplified by low molecular poly(ethylene oxide)) are also disclosed therein.

The article titled "Development and Evaluation of Highly-Loaded Coal Slurries" published in the 2nd International Symposium on Coal-Oil Mixture Combustion, Nov. 27-29, 1979, teaches coal-aqueous mixtures using coal of bimodal particle size distributions and containing modified starches, biocides and a wetting agent such as TRITON X, an octylphenoxy (ethyleneoxy) ethanol surfactant of low molecular weight.

And according to U.S. Pat. No. 3,617,095 a still further method is mentioned in the literature for forming emulsions of bulk solids by admixing the solid, such as coal, with water and oil in the presence of an oxyalkylated octyl phenol emulsifying agent.

Finally, a number of further patents disclose mechanical treatments and dispersants for providing coal in a carrier medium. See, e.g., U.S. Pat. Nos. 4,088,453; 4,104,035; 3,620,698; 3,764,547; 3,996,026; 3,210,168; 3,524,682; 4,330,301; 4,305,729; European Pat. No. 0050 412 and PCT International Application No. WO 81-01152.

While the art has attempted to provide coal in dispersed fluid form, as evidenced by the above-described procedures, there still remains the need for improving these methods in order to provide coal mixtures without undue mechanical or chemical treatment. It would be highly desirable to provide coal in aqueous mixture form wherein only minor amounts of additive materials are needed to disperse the coal to high solids concentrations of 70% by weight, or higher. It would be further desirable to provide coal-aqueous mixtures wherein the coal is precleaned of impurities so that the resultant

mixtures are clean burning or relatively clean burning and thus more environmentally acceptable.

### SUMMARY OF THE INVENTION

Accordingly, it is one object of the present invention to provide dispersions of coal in a carrier medium.

It is another object of the present invention to provide coal-aqueous mixtures of high coal solids content.

It is a further object of the invention to provide coal-aqueous mixtures of high solids content wherein only minor amounts of additive materials are needed and little mechanical treatment is required. 10

It is still another object of the present invention to provide coal-aqueous mixtures of high solids content which employ less costly additive materials than heretofore utilized. 15

It is still a further object of the invention to provide coal-aqueous mixtures wherein the dispersed coal is precleaned of impurities so that the resultant mixtures are clean-burning or relatively clean-burning. 20

A further object of the invention is to provide suitable methods for forming coal-aqueous mixtures.

These and other objects will become apparent from the accompanying detailed description. 25

### DETAILED DESCRIPTION OF THE INVENTION

U.S. Ser. No. 230,062 filed Jan. 29, 1981, now U.S. Pat. No. 4,358,293, incorporated herein by reference discloses the surprising discovery that certain polyalkyleneoxide nonionic surfactants are excellent additives for forming coal-aqueous mixtures having high coal solids concentrations. It is disclosed therein that polyalkyleneoxide nonionic surfactants of high molecular weight having a hydrophobic portion and a hydrophilic portion, the hydrophilic portion being comprised of at least about 100 ethylene oxide repeating units, provide coal-water dispersions having very high coal solids concentrations of about 70% by weight coal, or higher, when the surfactant is present in an amount sufficient to 30 disperse the particulate coal in water. The resultant mixtures are free-flowing and are adapted to provide coal in a form ready for transport, storage and clean-burning. Surprisingly, the surfactants employed can differ in chemical structure so long as they are of the 45 selected type, are of sufficient molecular weight and are comprised of at least about 100 units of ethylene oxide.

Copending U.S. Ser. No. 416,006 filed Sept. 10, 1982 incorporated herein by reference discloses that by employing certain processing conditions, in the preparation of the coal-aqueous slurries disclosed in the aforementioned U.S. application Ser. No. 230,062, (now U.S. Pat. No. 4,358,293) even more improved coal-aqueous slurries are provided.

It has now been surprisingly discovered that by employing a combination of the polyalkyleneoxide nonionic surfactants of said U.S. Ser. No. 230,062 (now U.S. Pat. No. 4,358,293) and a polyelectrolyte dispersing agent, such as an oligomeric polyacrylate anionic surfactant, high solids content coal-aqueous slurries are 55 also obtained. Thus, in accordance with the present invention, less costly nonionic surfactant need be employed while still obtaining the same high solids content of the coal slurry.

Thus, the coal-aqueous slurries of the present invention are comprised of coal or other carbonaceous material as the dispersed solid; water as the carrier medium; and a combination of a polyalkyleneoxide nonionic 60

surfactant, as further described herein and a polyelectrolyte dispersing agent, such as a polycarboxylic acid, preferably an oligomeric (low molecular weight polymer) anionic polyacrylate surfactant, as also further described herein.

As used herein "polyalkyleneoxide nonionic surfactant" connotes all compositions, compounds, mixtures, polymers, etc. having in part an alkylene oxide repeating unit of the structure:



and having a hydrophobic portion and a hydrophilic portion and which does not dissociate or ionize in solution. These surfactants have a polymeric portion comprised of repeating units of ethylene oxide of the general formula:



Moreover, the polyalkyleneoxide nonionic surfactant compositions employed in this invention are of high molecular weight, i.e., from about 4,000 or higher, depending on the particular surfactant employed, are hydrophilic and are comprised of at least about 100 repeating units of the ethylene oxide monomer. In addition, the surfactants utilized have a hydrophobic portion and a hydrophilic portion and are nonionic. Being nonionic, these compositions are generally not subject to ionization in aqueous solutions of acid or alkali.

Suitable hydrophilic polyalkyleneoxide nonionic surfactants for use in this invention are the commercially available glycol ethers of alkyl phenols of the following general formula I:



wherein R is substituted or unsubstituted alkyl of from 1 to 18 carbon atoms, preferably 9 carbon atoms; substituted or unsubstituted aryl, or an amino group and n is an integer of at least about 100.

These nonionic surfactants are available in a wide array of molecular weights depending primarily on the value of "n", i.e., the number of ethylene oxide repeating units. Surprisingly, it has been found that these surfactants of a high molecular weight of about 4,000 or higher wherein "n" is at least 100, or higher are particularly effective as dispersants for forming coal-aqueous mixtures to high coal solids concentration requiring little if any further additives, etc., to form highly flowable liquids.

Procedures for the preparation of the glycol ethers of formula I are well known and are described, for example, in U.S. Pat. Nos. 2,213,477 and 2,496,582, which disclosures are incorporated herein by reference. Generally, the production of these compositions involves the addition of substituted phenols with molar proportions of ethylene oxide monomer.

Thus, polyalkyleneoxide nonionic surfactants suitable for use in the invention include the glycol ethers of alkylated phenols having a molecular weight of at least about 4,000 of the general formula:



wherein R is substituted or unsubstituted alkyl of from 1 to 18 carbon atoms, preferably 9 carbon atoms; substituted or unsubstituted aryl, or an amino group, and n is an integer of at least about 100. The substituents of the alkyl and aryl radicals can include halogen, hydroxy, and the like.

Other suitable nonionic surfactants are the poly(oxyethylene)-poly(oxypropylene)-poly(oxyethylene) or, as otherwise described, propoxylated, ethoxylated propylene glycol nonionic surfactant block polymers having a molecular weight of at least about 6,000 of the general formula:



wherein a, b and c are whole integers and wherein a and c total at least about 100.

Still other polyalkyleneoxide nonionic surfactants suitable for use in the invention are the block polymers of ethylene and propylene oxide derived from nitrogen-containing compositions such as ethylene diamine and having a molecular weight of at least about 14,000 of the general formula:



wherein R<sub>1</sub> is an alkylene radical having from 2 to 5 carbon atoms, preferably 2; R<sub>2</sub> is alkylene radical having 3 to 5 carbon atoms, preferably 3; a, b, c, d, e, f, g and h are whole integers; and e, f, g and h total at least about 100.

The most preferred glycol ethers of the type generally described in formula I are the nonylphenoxy (polyethoxylated) ethanol compositions of the formula:



wherein n is about 100 or higher.

Commercially available surfactants of this type are supplied by the GAF Corporation under the designations IGEPAL CO-990 and IGEPAL CO-997. Other commercially available surfactants of this type are supplied by the Thompson-Hayward Chemical Co. under the designation T-Det N-100, and Whitestone Chemical Co. under the designation ICONOL NP-100.

As stated hereinbefore, another group of polyalkyleneoxide nonionic surfactants useful in the invention are the well known poly(oxyethylene)-poly(oxypropylene)-poly(oxyethylene) nonionic surfactant block polymers. These surfactants comprise the block polymers of ethylene oxide and propylene oxide with the repeating units of propylene oxide constituting the

hydrophobic portion of the surfactant; and the repeating units of ethylene oxide constituting the hydrophilic portion of the surfactant. These block polymer compositions are of the general formula II:



wherein a, b and c are whole integers and wherein a and c total at least about 100.

These compositions can be prepared, and are commercially available, in a variety of molecular weights, depending primarily on the number of repeating units of propylene and ethylene oxide. It has been found that these block polymers having a molecular weight of at least about 6,000 and comprising at least about 100 repeating units of ethylene oxide are excellent additives for dispersing coal in a water carrier to the desired high coal solids concentrations of about 45 to 80 percent, preferably about 70 percent coal particles, based on the weight of the total mixture. Thus, with reference to the above formula II, the poly(oxyethylene)-poly(oxypropylene)-poly(oxyethylene) nonionic surfactants suitable for use in the invention are those wherein a, b and c are integers and a and c total about 100 or higher.

Suitable procedures for the production of the block polymers of Formula II are described in the patent literature in, for example, U.S. Pat. Nos. 2,674,619; 2,677,700 and 3,101,374, which are incorporated herein by reference.

Generally, these block polymers are prepared by a controlled addition of propylene oxide to the two hydroxyl groups of propylene glycol to form the hydrophobe, followed by the controlled addition of ethylene oxide to "sandwich" in the hydrophobe between the two hydrophilic polyethoxylate groups.

The nonionic surfactants of this type (Formula II) having the requisite number of at least 100 units of ethylene oxide are available from the BASF-Wyandotte Corporation under the PLURONIC designation, Series Nos. F-77, F-87, F-68, F-88, F-127, F-98, and F-108. These compositions have at least 100 ethylene oxide units, as per the following table of these PLURONIC surfactants:

| PLURONIC F | Mol. Wt. | Number of Ethylene Oxide Units |                                |
|------------|----------|--------------------------------|--------------------------------|
|            |          | % Ethylene Oxide               | Number of Ethylene Oxide Units |
| F-77       | 6,600    | 70                             | 105                            |
| F-87       | 7,700    | 70                             | 120                            |
| F-68       | 8,350    | 80                             | 151                            |
| F-88       | 10,800   | 80                             | 195                            |
| F-127      | 12,500   | 70                             | 200                            |
| F-98       | 13,000   | 80                             | 235                            |
| F-108      | 14,000   | 80                             | 255                            |

As also described hereinbefore, a further group of polyalkyleneoxide nonionic surfactants suitable as coal dispersants herein are the nitrogen containing block polymers of the general formula III:



wherein R<sub>1</sub> is an alkylene radical having 2 to 5 carbon atoms, preferably 2; R<sub>2</sub> is an alkylene radical having 3 to

5 carbon atoms, preferably 3; a, b, c, d, e, f, g and h are whole integers; and e, f, g and h total at least about 100.

These materials are prepared by the addition of a C<sub>3</sub> to C<sub>5</sub> alkylene oxide to an alkylene diamine under conditions to add two polyoxyalkylene groups to each of the nitrogen groups in the presence of a catalyst so as to polymerize the oxyalkylene groups into the desired long-chained polyoxyalkylene radicals. After the desired addition and polymerization of the C<sub>3</sub> to C<sub>5</sub> alkylene oxide group has been completed, ethylene oxide is introduced and is added to the polyoxyalkylene groups to impart the desired hydrophilic characteristics to the compound. The preparation of these materials from commercially available alkylene diamines and alkylene oxides is known in the art.

In general, the agents are prepared by mixing the C<sub>3</sub> to C<sub>5</sub> alkylene oxide with the alkylene diamine at atmospheric or elevated pressures, at temperatures between about 50° to 150° centigrade and in the presence of an alkaline catalyst such as an alkali metal hydroxide or alcoholate. The degree of polymerization or the size of the hydrophobic group is controlled by the relative proportions of C<sub>3</sub> to C<sub>5</sub> alkylene oxide and alkylene diamine, the alkylene oxide being introduced in a sufficient quantity to obtain a hydrophobic base weight of about 2000 to 3600 units although other weights can be provided.

These surfactants (Formula III) having the requisite number of at least 100 ethylene oxide repeating units are available from the BASF Wyandotte Chemicals Corporation under the TETRONIC designations Series Nos. 1107; 1307; 908 and 1508. These compositions have at least 100 ethylene oxide units, as per the following table of these TETRONIC surfactants.

| TETRONIC | Mol. Wt. | % Ethylene Oxide | Number of Ethylene Oxide Repeating Units |
|----------|----------|------------------|------------------------------------------|
| 1107     | 14,500   | 70               | 230                                      |
| 1307     | 15,500   | 70               | 245                                      |
| 908      | 16,500   | 80               | 300                                      |
| 1508     | 17,000   | 80               | 309                                      |

The anionic surfactants utilized in combination with the heretofore-identified nonionic surfactants are generally polyelectrolyte dispersing agents, such as polycarboxylic acid salts, preferably polyacrylates. Thus, examples of suitable polyelectrolyte dispersing agents useful herein include alkali metal and ammonium salts of polycarboxylic acids, such as for instance polyacrylic acid. Particularly preferred polycarboxylic acids are the 50 oligomeric anionic polyacrylate surfactants, such as for example those known as Polywet 67B (an oligomeric polyacrylate having a molecular weight of about 5000, available from Uniroyal Chemical Company), Nopcosperse 44 (anionic polyelectrolyte, available from Diamond Shamrock), DISPEX N-40 (a salt of a polycarboxylic acid, available from Allied Colloids), Polywet ND-2 (a sodium salt of a functional oligomer, available from Uniroyal Chemical Company). Anionic surfactants of this type are disclosed for example in U.S. Pat. No. 4,217,109 and European Patent Application No. 0,041,337 both of which are incorporated herein by reference.

The coal-aqueous mixture compositions of the invention herein are characterized by having a high coal solids content and a relatively low viscosity of about 2,000 or lower to in excess of 6,000 centipoise (cP) as measured e.g., in a Brookfield viscometer, model

#RVT, fitted with a number 3 spindle, at 100 r.p.m. even at solids levels of 70% by weight, or higher, based on the total weight of the mixture. These compositions can also include amounts of conventional flow modifying materials, such as thickeners, glues, defoaming agents, salts, etc., depending upon the use intended.

The products of the invention contain only minor amounts of surfactant additives in the order of about 0.1 to 3.0 percent by weight (total surfactant) of the total composition. Generally, the nonionic component is present in amounts from about 0.36 to about 0.57% by weight of dry coal and the anionic component in amounts from about 0.04 to 0.16% by weight of the dry coal. The products of this invention further contain particulate coal as the dispersed solid in an amount from about 45 to 80 percent; water as the carrier medium in an amount of from about 19.9 to 52 percent and, if desired, from about 0.1 to 2 percent of a thickener or thickeners; about 0.1 to 2 percent of a defoaming agent and about 0.1 to 2 percent of salts, anti-bacterial agents, caustic or other additive flow control agents, all of the percentages given being based on the total weight of the mixture.

Any of a wide array of coals can be used to form the coal-aqueous mixtures of this invention, including anthracite, bituminous, sub-bituminous, mine tailings, fines, lignite and the like. Other finely divided solid carbonaceous materials may also be used, e.g., coke, prepared either from coal or from petroleum.

To form the coal-aqueous mixtures, coal is pulverized to approximately 90% finer than a 200 mesh Tyler Standard screen size, although courser or finer particle sizes can be employed, if desired. A preferred particle size distribution is disclosed in U.S. Ser. No. 495,627 filed concurrently herewith incorporated by reference herein.

Advantageously, according to the invention, the untreated pulverized raw coal, is beneficiated, i.e., cleaned of amounts of ash and sulfur. The art will appreciate that mixtures formed of beneficiated coal offer considerable advantage. They are clean burning or relatively clean burning, and are more suited for burning in apparatus for powering utilities, home burners and the like without undue burdensome and expensive cleaning apparatus.

Any of a wide array of beneficiating treatments can be employed in preparing the particulate coals, including conventional heavy-media separations, magnetic separation and the like. The preferred method for providing the beneficiated coal particles is by a chemical treatment process such as described in U.S. Pat. No. 4,304,573.

Generally, according to the preferred chemical beneficiation treatment method, raw as-mined coal is ground in the presence of water to a particle size of about 200 mesh. The ground coal is treated in an aqueous medium with a monomeric compound, generally an unsaturated polymerizable composition such as readily available tall oil fatty acids in the presence of a metal initiator such as cupric nitrate; and minor amounts of fuel oil, all in an aqueous phase are also present. The ground coal so treated is made hydrophobic and oleophilic and is separated from the unwanted ash and sulfur by a froth flotation technique.

The cleaned coal recovered from the preferred chemical treatment process, now in the form of beneficiated coal particles, is suited for the coal-aqueous mixtures of

the invention. These coal particles are characterized by having an ash content reduced to levels of about 0.5 to 6.0% and a sulfur content reduced to levels of about 0.5 to 2.0%.

In one method herein the coal-aqueous mixtures can be prepared by first adding the surfactants to water together with other additives such as conventional defoaming agents, if desired. This admixing can be done with stirring at conditions of atmospheric or nearly atmospheric temperature and pressure. Thereafter, the particulate coal, preferably beneficiated coal particles, is added to the mixture to produce a coal-aqueous mixture of high coal solids content of about 45 to 80% by weight coal, based on the total weight of the mixture at atmospheric or nearly atmospheric temperatures and pressures. If desired, thickeners can then be added to further stabilize the mixture to assist in preventing the coal particles from settling when the mixture is to be stored for extended periods. Caustic soda or other bases can also be added at this point. As will be apparent, adding thickeners in or near the final stage is preferred so that the stirring requirements are kept at a minimum. The coal-aqueous mixtures can be prepared in a batch operation or in the continuous mode. In continuous production, the coal can be admixed with water in a first stage along with other flow control agents such as the surfactants. The compositions of the first stage can then be transferred continuously to a second stage wherein the thickener is added. Again, adding the thickener at the later stage results in reduced stirring requirements.

A preferred method for preparing the coal-aqueous compositions of the present invention, involves first adding the surfactants (nonionic and anionic) and other additives such as conventional defoaming agents, if desired, to water and mixed, under low speed agitation conditions, such as at from about 500 rpm to about 1500 rpm, preferably about 1000 rpm, for a time of from about 30 seconds to about 3 minutes, preferably about 1 minute. Thereafter, the particulate coal, preferably beneficiated coal particles, is added to the mixture and admixing therein under moderate or medium agitation conditions, for example, at an rpm in the range of from about 1000 rpm to about 3000 rpm, preferably about 2000 rpm for a time sufficient to provide a wetted out admixture. Usually this time is in the range of from about 5 minutes to about 20 minutes. At this time, the

15 minutes, preferably about 10 minutes. If desired, thickeners are then added to the slurry under the aforescribed high speed agitation conditions, e.g. 4000 rpm, for a further time of from about 1 minute to about 3 minutes, preferably about 2 minutes. In the preparation of a most preferred formulation, other ingredients, such as viscosity stabilizers such as ammonia and anti-bacterial agents such as formaldehyde are then added to the formulation at high speed agitation for a further time of from about 1 minute to about 3 minutes, preferably about 2 minutes. By wetted out or wet as used herein, it is meant that the surface of each coal particle is covered with water.

Typical mixing or dispersing apparatus employed herein include for example Premier Mill Co.'s Hi-Vi-  
persator High-Speed Disperser.

The above indicated residence times, temperatures, mixing speeds, etc. may vary according to specific process requirements such as the volume of ingredients, size of apparatus, mixing efficiency, etc. Thus, for example, depending on the scale of the operation, e.g., pilot plant, plant, etc., these process conditions of the present invention may be adjusted accordingly.

As indicated above, additives that can be added to the coal-aqueous mixture include defoaming agents, thickeners, salts, bases, other flow modifying agents and combinations of these materials.

Generally, the defoaming agents that can be used are conventional and include both silicon and non-silicon containing compositions. A commercially available defoaming agent suitable for use in the mixtures is COLLOID 691, supplied by Colloids, Inc. This composition generally comprises a mixture containing mineral oil, amide and an ester.

Thickeners can also be added to the mixture. They are added to increase the non-settling characteristics of the composition. Suitable thickeners include, for example xanthan gum, guar gum, glue and the like. Other thickeners include, for example, alkali soluble acrylic polymers (e.g. ACRYSOL ICS-1 sold by the Rohm and Haas Company). Combinations of these thickeners are also contemplated herein. For the purposes herein, the thickeners are generally used in amounts ranging from about 0.01 to about 3.0% by weight, based on the total weight of the mixture.

The following examples will further illustrate the invention:

| Ingredient (parts by weight) | Example |       |       |       |       |       |
|------------------------------|---------|-------|-------|-------|-------|-------|
|                              | 1       | 2     | 3     | 4     | 5     | 6     |
| 1. Clean Coal                | 244.0   | 244.0 | 244.0 | 244.0 | 244.0 | 244.0 |
| 2. Water                     | 104.0   | 104.0 | 104.0 | 104.0 | 104.0 | 104.0 |
| 3. Tetronic 1307             | 1.2     | 1.0   | 1.2   | 1.0   | 1.2   | 1.0   |
| 4. Polywet 67B               | —       | 0.2   | —     | 0.2   | —     | 0.2   |
| 5. Colloid 691               | 0.1     | 0.1   | 0.1   | 0.1   | 0.1   | 0.1   |
| 6. Guar Gum                  | 0.3     | 0.3   | 0.3   | 0.3   | 0.35  | 0.35  |
| 7. Kelzan                    | 0.05    | 0.05  | 0.05  | 0.05  | 0.05  | 0.05  |
| 8. 28% NH <sub>3</sub>       | 0.5     | 0.5   | 0.5   | 0.5   | 0.5   | 0.5   |
| 9. 37% CH <sub>2</sub> O     | 0.5     | 0.5   | 0.5   | 0.5   | 0.5   | 0.5   |
| Viscosity cP                 |         |       |       |       |       |       |
| Before Thickener             | 620     | 610   | 594   | 413   | 610   | 790   |
| 100 RPM                      |         |       |       |       |       |       |
| After Thickener              | 3200    | 4500  | 4600  | 5860  | 2500  | 3400  |

agitation of the admixture is increased to a high speed, 65 for example, from above about 3000 rpm to about 6000 rpm, preferably about 4000 rpm for a time sufficient to disperse the coal, usually from about 5 minutes to about

The three pairs of examples illustrated above show that in each comparison a combination of 1.0 grams of

Tetronic 1307 and 0.2 grams of Polywet 67B gave equal or better viscosity values (lower unthickened viscosity and higher thickened viscosity) indicating more complete dispersion of the coal compared to the samples that used Tetronic 1307 (1.2 grams) alone. Settling examination showed an advantage for the samples with the surfactant combination.

Identification of Ingredients

1. Wells Blend MF Clean Coal
2. Industrial Water
3. nonionic surfactant—BASF Wyandotte Corp.
4. anionic surfactant—Uniroyal Chemical Company
5. anti-foam agent—Colloids, Inc.
6. Guar Gum—Hercules
7. Xanthan Gum—Kelco Division, Merck & Co., Inc.
8. ammonium hydroxide—Fischer Scientific
9. formaldehyde solution—Borden Chemicals

Having fully described an embodiment of the foregoing invention, it is to be understood that this description is offered by way of illustration only. The range of adaptability of the invention presented herein is contemplated to include many variations and adaptations of the subject matter within the scope of the production of coal-aqueous mixtures. And it is to be understood that this invention is to be limited only by the scope of the appended claims.

I claim:

1. A stabilized, high solids content coal-aqueous mixture comprising particulate coal as a dispersed solid material; water as a carrier medium; a polyalkyleneoxide nonionic surfactant having a hydrophobic portion and a hydrophilic portion, said hydrophilic portion comprising at least about 100 units of ethylene oxide and a polyelectrolyte surfactant, said polyalkyleneoxide nonionic surfactant and said polyelectrolyte surfactant being present in said mixture in an amount sufficient to disperse said particulate coal in said water carrier.
2. The stabilized, high solids content coal-aqueous mixture of claim 1 wherein said polyelectrolyte surfactant is an oligomeric anionic polyacrylate.
3. The stabilized, high solids content coal-aqueous mixture of claim 1 further comprising a viscosity stabilizer.
4. The stabilized, high solids content coal-aqueous mixture of claim 1 further comprising a thickening agent.
5. The stabilized, high solids content coal-aqueous mixture of claim 1 further comprising an anti-foam agent.
6. The stabilized, high solids content coal-aqueous mixtures of claim 1 further comprising a thickening agent and an anti-foam agent.
7. The stabilized high solids content coal-aqueous mixtures of claim 1 wherein said polyalkyleneoxide nonionic surfactant has a high molecular weight at least about 4000.
8. The stabilized, high solids content coal-aqueous mixture of claim 1 wherein said polyalkyleneoxide nonionic surfactant comprises a composition of the formula



wherein R is substituted or unsubstituted alkyl of from 1 to 18 carbon atoms; substituted or unsubstituted aryl or an amino group, and n is an integer of at least about 100.

5 9. The stabilized, high solids content coal-aqueous mixture of claim 8 wherein R is a nonyl.

10. The stabilized, high solids content coal-aqueous mixture of claim 8 wherein said polyalkyleneoxide nonionic surfactant has a molecular weight of at least about 4000.

11. The stabilized, high solids content coal-aqueous mixture of claim 1 wherein said polyalkyleneoxide nonionic surfactant comprises a composition of the formula



wherein a, b and c are whole integers and a and c total at least about 100.

20 12. The stabilized, high solids content coal-aqueous mixture of claim 11 wherein said polyalkyleneoxide nonionic surfactant has a molecular weight of at least about 6000.

25 13. The stabilized, high solids content coal-aqueous mixture of claim 1 wherein said polyalkyleneoxide nonionic surfactant comprises a composition of the formula



35 wherein R<sub>1</sub> is an alkylene radical having 2 to 5 carbon atoms; R<sub>2</sub> is an alkylene radical having 3 to 5 carbon atoms; a, b, c, d, e, f, g and h are whole integers and e, f, g and h total at least about 100.

40 14. The stabilized, high solids content coal-aqueous mixture of claim 13 wherein R<sub>1</sub> is an alkylene radical having 2 carbon atoms and R<sub>2</sub> is an alkylene radical having 3 carbon atoms.

15. The stabilized, high solids content coal-aqueous mixture of claim 2 wherein said viscosity stabilizer comprises ammonia.

45 16. A method for forming a coal-aqueous mixture comprising admixing particulate coal with water, a polyalkyleneoxide nonionic surfactant having a hydrophobic portion and a hydrophilic portion, said hydrophilic portion being comprised of at least about 100 units of ethylene oxide and a polyelectrolyte surfactant.

50 17. The method of claim 16 wherein said polyelectrolyte surfactant is an oligomeric anionic polyacrylate.

18. The method of claim 16 wherein said polyalkyleneoxide nonionic surfactant is of the general formula:



wherein R is a substituted or unsubstituted alkyl of from 1 to 18 carbon atoms; substituted or unsubstituted aryl or an amino group and n is an integer of at least about 100.

65 19. The method of claim 16 wherein said polyalkyleneoxide nonionic surfactant is of the formula:



wherein a and c are whole integers totaling at least about 100.

20. The method of claim 16 wherein said polyalkyleneoxide nonionic surfactant is of the formula:



wherein  $\text{R}_1$  is an alkylene radical having 2 to 5 carbon atoms;  $\text{R}_2$  is an alkylene radical having 3 to 5 carbon atoms; a, b, c, d, e, f, g and h are whole integers and e, f, g and h total at least about 100.

21. The method of claim 16 wherein a thickening agent is added to said coal-aqueous mixture.

22. The method of claim 16 wherein said thickening agent is selected from the group consisting of xanthan gum, guar gum, cellulose gum, glue and alkali soluble acrylic polymer.

23. The method of claim 16 wherein a defoaming agent is added to said coal-aqueous mixture.

24. The method of claim 23 wherein said defoaming agent comprises a mixture of mineral oil, amide and polyethylene glycol oleate ester.

25. The method of claim 16 wherein a salt is added to said coal-aqueous mixture.

26. The method of claim 16 wherein said salt is sodium chloride.

27. The method of claim 16 wherein a caustic is added to the mixture.

28. The method of claim 16 wherein said coal-aqueous mixture is prepared in a continuous operation.

29. The method of claim 28 wherein said continuous operation for preparing said coal-aqueous mixture comprises first admixing said particulate coal with said water and said polyalkyleneoxide nonionic surfactant and an oligomeric polyacrylate anionic surfactant in a first stage and thereafter adding a thickener in a second stage.

30. The method of claim 16 wherein  $\text{NH}_4\text{OH}$  is added to said coal aqueous mixture.

31. A method for forming a coal-aqueous mixture, said method comprising the steps of:

- (i) admixing a polyalkyleneoxide nonionic surfactant having a hydrophobic portion and hydrophilic portion, said hydrophilic portion being comprised of at least about 100 units of ethylene oxide and a polyelectrolyte surfactant, with water, under low speed agitation conditions;
- (ii) admixing particulate coal with the admixture resulting from step (i) under medium speed agitation conditions; and
- (iii) agitating the resultant coal containing mixture of step (ii) under high speed agitation.

32. The method of claim 31 wherein said polyelectrolyte surfactant is an oligomeric anionic polyacrylate.

33. The method of claim 31 wherein said medium speed agitation in step (ii) is carried out for a time sufficient to wet the coal particles and said high speed agitation is carried out for a time sufficient to disperse the coal.

34. The method of claim 31 wherein an anti-foam agent is added to the mixture during step (i).

35. The method of claim 31 including the further steps of:

(iv) admixing a thickening agent under high speed agitation conditions, to the admixture resulting from step (iii).

36. The method of claim 35 wherein said thickening agent is selected from the group consisting of xanthan gum, guar gum, cellulose gum, glue and alkali soluble acrylic polymer.

37. The method of claim 33 wherein said anti-foam agent is comprised a mixture of mineral oil, amide and polyethylene glycol oleate ester.

38. The method of claim 35 including the further step of:

(v) admixing a member selected from the group consisting of an anti-bacterial agent, a viscosity stabilizer and mixtures thereof to the mixture resulting from step (iv), under high speed agitation.

39. The method of claim 38 wherein said viscosity stabilizer is ammonia.

40. The method of claim 31 wherein said particulate coal is added in an amount from about 45 to 80 percent; said water is added in an amount from about 19.9 to 52 percent; said polyalkyleneoxide nonionic surfactant is added in an amount from about 0.36 to about 0.57 percent, based on the weight of dry coal and said polyelectrolyte surfactant is added in an amount of from about 0.04 to about 0.16% by weight of the dry coal.

41. The method of claim 31 wherein said polyalkyleneoxide nonionic surfactant has a molecular weight of at least about 4000.

42. The method of claim 31 wherein said polyalkyleneoxide nonionic surfactant comprises a composition of the formula



45. wherein R is substituted or unsubstituted alkyl of from 1 to 18 carbon atoms; substituted or unsubstituted aryl or an amino group, and n is an integer of at least about 100.

43. The method of claim 42 wherein R is nonyl.

44. The method of claim 42 wherein said polyalkyleneoxide nonionic surfactant has a molecular weight of at least about 4000.

45. The method of claim 31 wherein said polyalkyleneoxide nonionic surfactant comprises a composition of the formula



60. wherein a, b and c are whole integers and a and c total at least about 100.

46. The method of claim 45 wherein said polyalkyleneoxide nonionic surfactant has a molecular weight of at least about 6000.

47. The method of claim 31 wherein said polyalkyleneoxide nonionic surfactant comprises a composition of the formula



wherein  $\text{R}_1$  is an alkylene radical having 2 to 5 carbon atoms;  $\text{R}_2$  is an alkylene radical having 3 to 5 carbon atoms;  $a, b, c, d, e, f, g$  and  $h$  are whole integers and  $e, f, g$  and  $h$  total at least about 100.

48. The method as defined in claim 47 wherein  $\text{R}_1$  is an alkylene radical having 2 carbon atoms and  $\text{R}_2$  is an alkylene radical having 3 carbon atoms.

49. The method of claim 35 where said thickening agent is added in an amount to result in from about 0.01 to 3 percent by weight of the total mixture.

50. The method of claim 31 wherein said particulate coal is beneficiated.

51. The method of claim 31 wherein said particulated coal is about 200 mesh in Tyler Standard screen size.

52. The method of claim 31 wherein said particulate coal is characterized by having a sulfur content of from 0.5 to 2.0 percent by weight, and an ash content of from about 0.5 to 6.0 percent, based on the weight of dry coal.

53. The method of claim 52 wherein said particulate coal further includes a fuel oil.

15 54. The method of claim 31 wherein said particulate coal is non-beneficiated.

\* \* \* \* \*

20

25

30

35

40

45

50

55

60

65

UNITED STATES PATENT AND TRADEMARK OFFICE  
CERTIFICATE OF CORRECTION

PATENT NO. : 4,478,603

DATED : October 23, 1984

INVENTOR(S) : Seymour Mark

It is certified that error appears in the above-identified patent and that said Letters Patent are hereby corrected as shown below:

Column 3, Line 48, "416,006" should read

--416,606--.

Signed and Sealed this

Twenty-third Day of April 1985

[SEAL]

Attest:

DONALD J. QUIGG

Attesting Officer

Acting Commissioner of Patents and Trademarks